

Dec. 15, 1925.

1,565,683

J. G. SWAIN

METHOD AND APPARATUS FOR ELECTROPLATING

Filed Nov. 12, 1923



FIG. 1.

JOSEPH G. SWAIN.

By

A. R. Ely

Attorney

Patented Dec. 15, 1925.

1,565,683

# UNITED STATES PATENT OFFICE.

JOSEPH G. SWAIN, OF AKRON, OHIO, ASSIGNOR TO THE FIRESTONE STEEL PRODUCTS COMPANY, OF AKRON, OHIO, A CORPORATION OF OHIO.

## METHOD AND APPARATUS FOR ELECTROPLATING.

Application filed November 12, 1923. Serial No. 674,119.

To all whom it may concern:

Be it known that I, JOSEPH G. SWAIN, a citizen of the United States, and a resident of Akron, county of Summit, State of Ohio, 5 have invented certain new and useful Improvements in Methods and Apparatus for Electroplating, of which the following is a specification.

This invention relates to a process of 10 electroplating by which a coating of mercury or an admixture of mercury is obtained with the other metal deposited upon iron or steel objects. The process and apparatus are particularly designed to be used in conjunction with zinc plating or electro- 15 galvanizing on metal automobile rims or similar objects.

In the drawings:

Figure 1 is a longitudinal section of a 20 portion of a plating tank;

Figure 2 is a section thereof on the line 2—2 of Figure 3;

Figure 3 is a longitudinal section through 25 one of the anodes used in the process; and

Figure 4 is a section on the line 4—4 of Figure 3.

The process of the invention consists in applying to the metal article to be plated, in conjunction with the zinc plating, a suitable proportion of mercury. In the preferred operation of the process, this action 30 is performed in a "strike" tank, or as a preliminary step in the electroplating process, the usual coating or electroplating with zinc taking place after the "strike" coat 35 is applied. The process is performed by anodes of metallic mercury in conjunction with the zinc anodes, the electric current being passed through both of said anodes 40 so that a small proportion of mercury is carried over and deposited on the articles. This operation preferably is performed in an electrolyte containing a cyanide solution. The number of mercurial anodes 45 relative to the zinc anodes may be limited within suitable ranges so that the proper results are obtained.

In the drawings, 1 represents a tank for containing the electroplating solution 2 50 which is usually one of the well known cyanide solutions. The articles to be plated, here represented as rims 3 which form the cathodes, are in the particular apparatus shown, suspended from hooks 4 which are 55 arranged to be carried upon a moving chain

5. The rims are connected by means of brushes 6 to a conductor rail 7 mounted over the tank. The electric current passes through a conductor rail 8 at the side of the tank and through anodes suspended within 60 the solution to the rims and then out through the rail 7, as will be readily understood.

In the carrying out of the present invention two types of anodes are suspended within 65 the electrolyte. The greater number of the anodes are zinc bars or rods 10 suspended from the rails 8, while at intervals the mercury anodes are provided.

These mercury anodes are indicated by 70 the numeral 11 in Figures 1 and 2. Their construction is clearly described in Figures 3 and 4. They comprise rods 12 of copper or other suitable conducting material which for the major part of their length 75 are incased in an insulating sleeve or shell 13, preferably of hard rubber or glass. At the base of the rod is attached a hard rubber or glass bowl or cup 14, which is attached to the rod by means of an integral 80 cross bar 15 extending transversely of the cup. The metallic mercury is contained in the cup and is covered over by insulating sieve or screen 16, the apertures of which permit the dispersion of mercury into the 85 electrolyte.

The operation of the invention will be readily understood by those skilled in the art, and is not necessarily limited to strict conformance with the showing and description herein contained. Changes and modifications may be made as will be understood, without departing from the spirit of the invention.

What I claim is:

1. In a process of electroplating, the steps of subjecting the article to be electroplated to an electrolyte charged simultaneously from anodes of zinc and metallic mercury.

2. In a process of electroplating, the steps of subjecting the article to be electroplated to a "strike" coat in an electrolyte charged from anodes containing zinc and metallic mercury.

3. In a process of electroplating, the steps of subjecting the article to be plated to a cyanide electrolyte charged from anodes containing zinc and metallic mercury.

4. In a process of electroplating, the step of simultaneously charging the plating solu- 110

tion through metallic mercury and a second plating metal.

5. In a process of electroplating, the steps of submerging within the electrolyte a mass of metallic mercury and simultaneously passing an electric current through the mercury as an anode and also through an anode of metallic zinc.

6. In the process of electroplating ferrous objects with zinc, the step of obtaining a "strike" coat of mercury and zinc by subjecting metallic mercury within the bath to an electric current simultaneously with zinc as anodes and subsequently plating with zinc.

7. An apparatus for electroplating com-

prising a cup, means to suspend the cup within the electrolyte, and means for conducting current to the interior of the cup.

8. An apparatus for electroplating comprising a tank, a cup within the tank adapted to contain metallic mercury, a conductor rod extending to and terminating within the cup, and an insulating covering for the conductor to prevent electric contact with the body of the electrolyte.

9. An apparatus for electroplating comprising a tank for holding electrolyte, a cup within the tank, a conductor rod, an insulating sleeve about the rod, and a per- 30 forated cover over the cup.

JOSEPH G. SWAIN.